

# UNITED STATES PATENT OFFICE.

ALBERT H. HENDERSON, OF TOWSON, MARYLAND.

## MANUFACTURE OF STEEL.

1,378,861.

Specification of Letters Patent. Patented May 24, 1921.

No Drawing.

Application filed July 9, 1919. Serial No. 309,656.

To all whom it may concern:

Be it known that I, ALBERT H. HENDERSON, a citizen of the United States, residing at Towson, in the county of Baltimore and 5 State of Maryland, have invented new and useful Improvements in the Manufacture of Steel, of which the following is a specification.

This invention, which has reference to a 10 process of refining and cleansing and improving the quality of steel, in no wise interferes with any regular and approved formulæ employed in the manufacture of steel, and may be used in connection with known 15 modes of making it from pig and other metal, as by the basic open hearth, the acid open hearth, or the Bessemer process, or by what is known as the duplex or the triplex methods involving joint uses of such 20 modes.

The main or characteristic features of the present invention relate, first, to the production of a molten metal cleansed and purified from deleterious matter such as phosphorous, sulfur, etc., the gases from such substances being liberated and allowed to escape; and, secondly, to a treatment in a ladle or the like of a selected body of such 25 cleansed, purified and molten metal, whether produced under either of the methods or combined methods herein alluded to, whereby are effected certain elemental changes in the metal drawn to the ladle, adapting the metal poured therefrom for the molding of 30 ingots or other castings free from piping, blow holes and the like, and having great tenacity, bending qualities, and ultimate strength, fitting it for forging, rolling, machining, etc. The steel produced under my 35 invention is well qualified for resistance to severe strains and shocks, as in the impact of projectiles, or under conditions to which railroad rails are exposed.

My invention, broadly considered, consists, 40 first, in a treatment of the charge at any appropriate time previous to or after it has reached the molten state, and before the tapping, for purifying it from deleterious matter, and secondly, a treatment of the 45 molten metal, after the tapping, whereby it is given certain elemental changes adapting the metal for the act of molding.

Certain features of the present invention are described in my copending application 50 Serial No. 256,591, filed October 2, 1918, and in my allowed application Serial No.

277,749, filed February 18, 1919. In each of my said applications anhydrous borax with other elements is included; but in the use of certain grades of iron, scrap, etc., in the 60 furnace it has been found that borax alone is sufficient for the purposes mentioned and that the other elements used for the cleansing and refining in the furnace, as set forth in my said applications may be omitted. 65 The purpose of the present invention is to retain only borax to the exclusion of other substances enumerated in said applications for cleansing the metal from oxidation, or removing other injurious characteristics, 70 whereby to lessen the cost of treatment and at the same time effect beneficial results in the product previous to the pouring thereof to the ladle in which the final step of my invention is carried out. 75

Referring first to the treatment of the charge, which may be effected at any appropriate selected time as above mentioned, and under either a single or a complex system, I add to each ton of metal about four 80 pounds of anhydrous borax, more or less, for the purpose of cleansing and refining the same. This amount of borax is deemed to be about the minimum needed for one ton of metal of high or even average grade; but 85 for lower grades the amount of borax per ton of metal will be varied within limits defined by the quality of the charge.

The anhydrous borax in the quantity or quantities desired may be packed in a readily 90 combustible envelop or series of envelops or containers each consisting of a pasteboard holder placed in a box of extra dry wood free from rosins or other substances and lined with heavy paper. However, the borax need 95 not be so or otherwise inclosed, and whether or not packed when thrown at any suitable time into the metal will readily liberate itself into the body thereof. The properties of anhydrous borax as a cleanser and purifier of 100 metal, as a cleanser or remover of oxidation and rust from steel and iron, and for brightening metal are well known. I have found that it is also useful in suppressing the gases in the furnace and consequently preventing 105 blow holes.

The desired furnace treatment having been effected, either by the single, duplex or complex system, that is to say, the fusing having been accomplished, I now pour the molten 110 metal, elementally changed by the initial process described, into a ladle, and while it

is therein add thereto the required proportion of lead, preferably in ingots, say about six pounds, more or less, together with about one or two pounds of zinc, to one ton of metal. The zinc, however, may be omitted and the lead used alone. The proportions of each of the various ingredients employed may be varied in view of the diversified classes of iron, as pig, scrap, steel and iron 10 castings, etc., constituting the charge, my process allowing the use of any kind of metal ordinarily used in the conversion of iron into steel.

The successful results seem to arise from 15 the introduction of the lead or the lead and zinc to the ladle before or after the filling or partial filling thereof, or at any time before the metal is poured from the ladle into the mold. It is found that but little if any slag 20 remains in the bottom of the ladle after the pouring into the ingot mold or the casting pattern. The results of these operations are the production of an ingot with greatly reduced cavities, recesses or piping at its head.

Having thus described my invention, I 25 claim:—

1. In the production of steel for molding into ingots or castings, adding to the charge during the fusing anhydrous borax in the proportion of about four pounds to each ton 30 of metal.

2. In the production of steel for molding into ingots or castings, adding to the charge during the fusing anhydrous borax in the proportion of about four pounds to each ton 35 of metal, and thereafter adding to a selected body of such fused metal while in a ladle about six pounds of lead to one ton of metal.

3. In the production of steel for molding into ingots or castings, adding to the charge 40 during the fusing anhydrous borax in the proportion of about four pounds to each ton of metal, and thereafter adding to such fused body while in a ladle about six pounds of lead together with approximately one to two 45 pounds of zinc to one ton of metal.

In testimony whereof I affix my signature.  
ALBERT H. HENDERSON.